

June 16, 1964

U. BIRKHOLZ  
THERMOCOUPLE, PARTICULARLY FOR ELECTROTHERMIC  
COOLING, AND METHOD OF PRODUCING IT  
Filed April 23, 1959

3,137,593



Fig. 3



Fig. 1



Fig. 2

## 1

3,137,593

## THERMOCOUPLE, PARTICULARLY FOR ELECTRO-THERMIC COOLING, AND METHOD OF PRODUCING IT

Ulrich Birkholz, Nurnberg, Germany, assignor to Siemens-Schuckertwerke Aktiengesellschaft, Berlin-Siemensstadt and Erlangen, Germany, a corporation of Germany

Filed Apr. 23, 1959, Ser. No. 808,384

Claims priority, application Germany Apr. 26, 1958  
7 Claims. (Cl. 136—4)

My invention relates generally to thermocouples and, in a preferred aspect, to Peltier couples for the electric production of cold temperatures.

Among the materials known for use in thermocouples or Peltier couples are a group of substances of improved efficacy that possess a relatively high differential thermoelectric force together with relative low heat conductance, and hence are characterized by a small Wiedemann-Franz-Lorentz number (WFL-number). Examples of such substances are bismuth, antimony-tellurium alloys composed of the compounds  $\text{Bi}_2\text{Te}_3$  and  $\text{Sb}_2\text{Te}_3$ . The compositions heretofore known contain more bismuth than antimony or contain both elements in substantially equal or only slightly differing proportions.

It is an object of my invention to provide thermocouple compositions and manufacturing methods by means of which a still greater thermoelectric efficacy than heretofore attainable can be obtained.

To this end, and in accordance with a feature of my invention, at least one member of a thermocouple, particularly a Peltier couple for the production of cold, is made of a solid solution (mixed crystal) of the compounds  $\text{Bi}_2\text{Te}_3$  and  $\text{Sb}_2\text{Te}_3$  with an antimony content between 24 and 36 atom percent and a bismuth content between 4 and 16 atom percent. Such solid solutions constitute a ternary system of the form:



in which  $y$  denotes a value between 1.2 and 1.8. Particularly advantageous is a composition of 28 atom percent antimony and 12 atom percent bismuth, corresponding to a value of  $y=1.4$  in the foregoing ternary formula.

The invention is based upon the surprising experimental discovery that maximum efficacies are attained if the antimony and bismuth proportions are dimensioned as stated above. The advantages of thus dimensioning the constituents are apparent from the following tabulation which reveals, in particular, that maximum efficacy is achieved with a composition of 28 atom percent antimony and 12 atom percent bismuth. As a rule, the compositions according to the invention have p-type conductance. By combining such a p-conducting couple member with a second member consisting of  $\text{Bi}_2\text{Te}_3$  which is n-conductively doped by an AgI addition of about 0.1% by weight, a thermocouple is obtained which, when operating as a Peltier couple, possesses a total efficacy of  $2.1 \cdot 10^{-3}$  per  $^{\circ}\text{C}$ . which corresponds to a theoretically obtainable reduction in temperature of  $80^{\circ}\text{C}$ . (referring to a cold junction at  $0^{\circ}\text{C}$ ).

| Sb-                            | Bi- | $\alpha$<br>$\mu\text{v.}/^{\circ}\text{C.}$ | WFL-number:<br>$10^8 \text{ volt}^2/^{\circ}\text{C.}^2$ | $z \cdot 10^3$<br>$^{\circ}\text{C.}^{-1}$ |
|--------------------------------|-----|----------------------------------------------|----------------------------------------------------------|--------------------------------------------|
| Proportion in<br>Atom, percent |     | 3                                            | 4                                                        | 5                                          |
| 1                              | 2   |                                              |                                                          |                                            |
| 8                              | 32  | +202                                         | 8.5                                                      | 1.68                                       |
| 20                             | 20  | +153                                         | 4.65                                                     | 1.77                                       |
| 24                             | 16  | +146                                         | 3.55                                                     | 1.91                                       |
| 28                             | 12  | +146                                         | 3.14                                                     | 2.1                                        |
| 32                             | 8   | +136                                         | 3.06                                                     | 2.04                                       |
| 36                             | 4   | +108                                         | 2.67                                                     | 1.30                                       |

## 2

Column 1 of the table indicates the antimony content in atom percent. Column 2 indicates the bismuth component in atom percent. Column 3 indicates the differential thermoforce ( $\alpha$ ). Column 4 indicates the WFL-number  $\times 10^8$  and column 5 indicates the efficacy ( $z$ )  $\times 10^3$ . The efficacy is defined as:

10

$$z = \frac{\alpha^2 \cdot \sigma}{\kappa}$$

in which

15  $\alpha$  denotes the differential thermoforce,  
 $\sigma$  denotes the electric conductance, and  
 $\kappa$  denotes the heat conductance.

20 The efficacy value  $z$  is a direct measure for the applicability of a substance as a thermoelectric component, particularly with respect to the obtainable temperature difference in an electrothermic combination. The value  $z$  is also a measure of the power capacity in electrothermic cooling and in thermoelectric generation of electric current.

25 It will be noted that the value of  $z$  is a maximum with the composition containing 28 atom percent antimony and 12 percent bismuth.

30 For further information reference will be made to the drawing showing in FIGS. 1 and 2 two respective graphs and in FIG. 3 a schematic illustration of a Peltier couple according to the invention.

35 Referring to FIG. 3, there is denoted by 1 a couple member consisting of a solid solution of  $\text{Bi}_2\text{Te}_3$  and  $\text{Sb}_2\text{Te}_3$  corresponding to the formula  $\text{Bi}_{0.6}\text{Sb}_{1.4}\text{Te}_3$  and having p-type conductance. The second member 2 of the couple consists of  $\text{Bi}_2\text{Te}_3$  doped with about 0.1% by weight of silver iodide (AgI) and having n-type conductance. The two members 1 and 2 are joined, by a solder or fusion joint, with three blocks 3, 4, 5 of copper. These blocks have respective channels to be joined with the pipes of coolant circulation systems. The channels of blocks 4 and 5 are to be traversed by a liquid medium for the purpose of keeping them approximately at a given temperature. The channel of the junction block 3 is to be connected into a coolant circulation line for conveying cooled liquid to the cooler, evaporator or other component to be cooled or refrigerated. As mentioned above, 50 such a Peltier couple affords a maximum reduction of temperature of about  $80^{\circ}\text{C}$ .

55 The thermoelectric components of a thermocouple according to the invention can be made in accordance with any of the methods known for the manufacture of thermocouple materials. Particularly advantageous is a production according to the powder-metallurgical method as generally known, for example from German Patent 836,943. One way of employing such a method for the

60 purposes of the invention is to produce the solid solution from the compounds  $\text{Bi}_2\text{Te}_3$  and  $\text{Sb}_2\text{Te}_3$  by melting the respective constituents in stoichiometric proportions, then cooling and pulverizing the resulting solid solution, and thereafter processing the powdered substance in accordance with the powder-metallurgical method for shaping and sintering the thermocouple member to be produced.

65 According to another feature of my invention, the manufacture of the thermocouple member by a powder-metallurgical method is performed in such a manner as to adapt the thermoelectric properties to desired require-

ments by suitably dimensioning the sintering data, namely the grain size, the amount of pressure applied to the pulverulent material, the sintering temperature, the sintering time and the atmosphere in which the sintering is carried out. In this manner, the defect-electron (hole) concentration can be reduced. In other words, the method is preferably performed under sintering conditions chosen for obtaining optimum charge-carrier concentration. Meant by "optimum charge-carrier concentration" is the charge-carrier concentration that results in an electronic heat conductance ( $\kappa_{el}$ ) satisfying as closely as feasible the following equation known from the theory of the Peltier effect:

$$\alpha = 172 \left( 1 + \frac{\kappa_{el}}{\kappa_G} \right) \mu\text{v./}^\circ\text{C.}$$

wherein  $\kappa_G$  denotes the lattice thermal conductance.

For example, with the above-mentioned preferred composition containing 28 atom percent antimony and 12 atom percent bismuth,  $\alpha$ -values of 200 to 300  $\mu\text{v./}^\circ\text{C.}$  can be attained by varying the sintering temperature between 250° C. and 500° C., and varying the pressure force between 2 t./cm.<sup>2</sup> and 8 t./cm.<sup>2</sup>. The letter t. means a metric ton, which is 1000 kilograms. In this case the duration of the sintering process is 1 hour, and the grain size of the starting powder is below 60 microns. The  $\alpha$ -value of the molten material is 145  $\mu\text{v./}^\circ\text{C.}$

A marked improvement in the thermoelectric properties is obtained by adding up to 1% by weight of selenium to the solid solution described above.

The optimum amount of the selenium addition is about 0.6% by weight. Such addition, in an alloy system with the optimum y-value of 1.4, produces an increase in efficiency from about  $z=2.1 \times 10^{-3} \text{ }^\circ\text{C.}^{-1}$  up to  $z=2.6 \times 10^{-3} \text{ }^\circ\text{C.}^{-1}$ .

The effect of the additions made according to the invention is due to a reduction in the defect-electron concentration which results in an increase in differential thermoforce and hence in efficacy. As a result, the above-mentioned optimum of the differential thermoforce is approached to a still further extent.

The effect of a selenium addition upon the differential thermoforce and the efficacy of the system according to the invention, relating to a composition with the optimum y-value=1.4, is represented in the graphs shown in the drawing. FIG. 1 indicates the differential thermoforce ( $\alpha$ ) in dependence upon the selenium addition. FIG. 2 indicates the dependence of the efficacy value ( $z$ ) upon the selenium addition.

In the graph of FIG. 1, the abscissa indicates the conductance ( $\delta$ ) on a logarithmic scale in  $(\Omega \text{ cm.})^{-1}$ , and the ordinate indicates the differential thermoforce ( $\alpha$ ) in  $\mu\text{v./}^\circ\text{C.}$  The diagram indicates two curves which coincide in part. The full-line curve relates to measured values, the broken-line curve indicates theoretical values. The measuring points for additions of 0%, 0.5% and 1% selenium are indicated by blackened circles.

In FIG. 2, the abscissa indicates the conductance ( $\sigma$ ) in  $(\Omega \text{ cm.})^{-1}$ , and the ordinate indicates the efficacy value ( $z$ ) in  $^\circ\text{C.}^{-1} \times 10^3$ . The diagram shows a full-line curve based upon experimental results, and a broken-line curve based upon theoretical values. Indicated are the  $\alpha$ -values ( $\alpha=146$ , or 171, or 193) corresponding to the measuring points shown in FIG. 1 for the respective selenium contents of 0%, 0.5% and 1%. It is apparent that with a selenium addition of 0.6% by weight ( $\alpha=182$ ) an optimum efficacy of about  $2.6 \times 10^{-3}$  per  $^\circ\text{C.}$  is achieved.

I claim:

1. An apparatus for thermoelectric cooling, comprising a thermocouple and electric connections for passing a current therethrough, the thermocouple comprising two members of extrinsically conductive material electrically connected to each other to form a junction, one of said members having p-type conductance and being a solid solution of  $\text{Bi}_2\text{Te}_3$  and  $\text{Sb}_2\text{Te}_3$  having an antimony content between about 24 and 32 atom percent and a bismuth content between about 8 and 16 atom percent and having selenium dispersed in said solid solution in an amount of about 0.1 to 1.0% by weight of the total composition, said member being made by preparing a melt of said composition, causing the melt to solidify, pulverizing the resulting solid solution, and forming said member by pressing and sintering the powder at between about 250° and 500° C. and at a pressure between about 2 t./cm.<sup>2</sup> and 8 t./cm.<sup>2</sup>, the other member being  $\text{Bi}_2\text{Te}_3$  n-conductivity doped by addition of  $\text{AgI}$ .

2. An apparatus for thermoelectric cooling, comprising a thermocouple and electric connections for passing a current therethrough, the thermocouple comprising two members of extrinsically conductive material electrically connected to each other to form a junction, one of said members having p-type conductance and being a solid solution of  $\text{Bi}_2\text{Te}_3$  and  $\text{Sb}_2\text{Te}_3$  having an antimony content between about 24 and 32 atom percent and a bismuth content between about 8 and 16 atom percent and having selenium dispersed in said solid solution in an amount of about 0.1 to 1.0% by weight of the total composition, said member being made by preparing a melt of said composition, causing the melt to solidify, pulverizing the resulting solid solution, and forming said member by pressing and sintering the powder at between about 250° and 500° C. and at a pressure between about 2 t./cm.<sup>2</sup> and 8 t./cm.<sup>2</sup>, the other member being  $\text{Bi}_2\text{Te}_3$ .

3. An apparatus for thermoelectric cooling, comprising a thermocouple and electric connections for passing a current therethrough, the thermocouple comprising two members of extrinsically conductive material electrically connected to each other to form a junction, one of said members having p-type conductance and being a solid solution of  $\text{Bi}_2\text{Te}_3$  and  $\text{Sb}_2\text{Te}_3$  having an antimony content between about 24 and 32 atom percent and a bismuth content between about 8 and 16 atom percent and having selenium dispersed in said solid solution in an amount of about 0.1 to 1.0% by weight of the total composition, said member being made by preparing a melt of said composition, causing the melt to solidify, pulverizing the resulting solid solution, and forming said member by pressing and sintering the powder at between about 250° and 500° C. and at a pressure between about 2 t./cm.<sup>2</sup> and 8 t./cm.<sup>2</sup>, the other member being n-conductive  $\text{Bi}_2\text{Te}_3$ .

4. The method of producing a thermocouple member, which comprises the steps of melting the compounds  $\text{Bi}_2\text{Te}_3$  and  $\text{Sb}_2\text{Te}_3$  in the proportion required for an antimony content between 24 and 36 atom percent and a bismuth content between 4 and 16 atom percent, pulverizing the resulting solid solution, and forming the member by pressing and sintering at a temperature between 250° C. and 500° C. and a pressure between 2 t./cm.<sup>2</sup> and 8 t./cm.<sup>2</sup>.

5. The method of producing a thermocouple member, which comprises the steps of preparing a melt of the composition  $\text{Bi}_{2-y}\text{Sb}_y\text{Te}_3$  wherein  $y=1.2$  to  $1.8$ , adding selenium in an amount up to about 1.0% by weight of the total composition, causing the melt to solidify, pulverizing the resulting mixed crystal material, and forming the member by pressing and sintering the powder at a temperature between 250° C. and 500° C. and a pressure between 2 t./cm.<sup>2</sup> and 8 t./cm.<sup>2</sup>.

6. The method of producing a thermocouple member which comprises the steps of preparing a solid solution of the composition  $\text{Bi}_{0.6}\text{Sb}_{1.4}\text{Te}_3$ , pulverizing said solid solution, and forming the member from the powder by sintering it at a temperature between 250° C. and 500° C. 5 and a pressure between 2 t./cm.<sup>2</sup> and 8 t./cm.<sup>2</sup>.

7. The method of producing a thermocouple member, which comprises the steps of preparing a melt of the composition  $\text{Bi}_{0.6}\text{Sb}_{1.4}\text{Te}_3$  and adding selenium to the melt in an amount of about 0.6% by weight of the total composition, permitting the melt to solidify, pulverizing the solid material, and forming the member from the powder by sintering it at a temperature between 250° C. and 500° C. and a pressure between 2 t./cm.<sup>2</sup> and 8 t./cm.<sup>2</sup>. 10

## References Cited in the file of this patent

## UNITED STATES PATENTS

|           |            |                |
|-----------|------------|----------------|
| 2,597,752 | Salisbury  | May 20, 1952   |
| 2,602,095 | Faus       | July 1, 1952   |
| 2,762,857 | Lindenblad | Sept. 11, 1956 |
| 2,877,283 | Justi      | Mar. 10, 1959  |
| 2,886,618 | Goldsmid   | May 12, 1959   |
| 2,990,439 | Goldsmid   | June 27, 1961  |

## FOREIGN PATENTS

|           |         |              |
|-----------|---------|--------------|
| 1,054,519 | Germany | Apr. 9, 1959 |
|-----------|---------|--------------|